

Aug. 11, 1931.

H. MARMORSTEIN

1,818,729

PROCESS OF DECORATING ARTICLES OF POTTERY AND THE LIKE

Filed Nov. 1, 1929



*Heinrich Marmorstein*

INVENTOR.

BY *Ernest J. Michaelis*

ATTORNEYS.

## UNITED STATES PATENT OFFICE

HEINRICH MARMORSTEIN, OF CHICAGO, ILLINOIS

## PROCESS OF DECORATING ARTICLES OF POTTERY AND THE LIKE

Application filed November 1, 1929. Serial No. 404,181.

The invention relates to a process of ornamenting an article made of glass, pottery, porcelain, china-ware or the like in such a manner, that the article will appear to have veins painted on its surface with dull roman gold.

Heretofore a process has been known, by which the surface of such articles has been ornamented so that it received veins in bright gold and in order to ornament the article of dull roman gold, it was necessary not only to use expensive roman gold, but also to go to the labour and trouble of painting the veins one by one onto the article to be decorated.

15 The object of the present invention therefore is to provide a process by which it will become unnecessary to use the expensive roman gold but use the less expensive so called liquid bright gold, and by which it will be unnecessary to paint each vein by itself onto the article to be ornamented.

The drawing forming a part of this specification illustrates a vase decorated according to the present invention.

25 The process according to the present invention consists of the following steps:

An article to be treated is provided with a dull glazed surface. The process of providing such a surface is well known and does not 30 form a part of the present invention and is therefore not described in this specification.

The article to be decorated is then covered with a coat of so called liquid bright gold. This is the trade name for a solution of gold, 35 nitric acid, to which solution hydrochloric acid is added. Preferably 30 grams of gold are dissolved in 350 grams of nitric acid and to this solution 75 grams of hydrochloric acid are added. Care has to be taken to entirely 40 cover the surface to be decorated with the liquid bright gold. The article is then left to dry in the atmosphere and when the liquid gold is thoroughly air-dried the surface covered by the gold is provided with a coat of a 45 solution produced in the following manner:

One part of Epsom salt is mixed with two parts of a malt brew and this mixture is heated until the salt is dissolved entirely and at a 50 degree of heat which permits the hand of the

operator to come in contact with the liquid without being scalded.

The solution is then kept lukewarm and the air-dried coat of gold is then covered with a coat of this solution. It is necessary that this 55 second coat covers the whole surface painted previously with gold. Then the article is left again to dry in the atmosphere and when it is thoroughly dry, it is burned in a kiln at a liquid gold fire i. e. about 1500° Fahrenheit. 60 After being burned the article is left in the kiln for three hours in order to permit it to cool off very slowly. When the article is taken out of the kiln it will appear, that the 65 outer coat is practically burned to ashes, which may be washed off by bathing the article in lukewarm water and drying by and it will also appear, that the coat of liquid bright gold has been exploded so, that the whole 70 surface is now covered with veins, which appear to be painted on the surface with dull roman gold.

Having described my invention and how the same is to be performed, I claim as new and desire to secure by Letters Patent: 75

In a process of the class described the steps of covering an article having a dull glazed surface with a coat of so called liquid bright gold, drying said coat in the atmosphere, covering said gilded surface entirely with a coat 80 of a solution consisting of Epsom salt dissolved in beer, drying said second coat in the atmosphere, burning the article in a kiln at liquid gold fire, leaving the article for about three hours in the kiln for cooling, and bathing the article in lukewarm water. 85

In witness whereof I affix my signature.

HEINRICH MARMORSTEIN.

90

95

100